

March 4, 1930.

E. H. BUNCE ET AL

1,749,127

REDUCING ZINCIFEROUS MATERIALS CONTAINING LEAD

Filed Jan. 4, 1928



INVENTOR

Earl H. Bunce  
George T. Mahler  
BY

Gemmie, Davis, Marvin & Edmonds  
ATTORNEYS

## UNITED STATES PATENT OFFICE

EARL H. BUNCE AND GEORGE T. MAHLER, OF PALMERTON, PENNSYLVANIA, ASSIGNEES TO THE NEW JERSEY ZINC COMPANY, OF NEW YORK, N. Y., A CORPORATION OF NEW JERSEY

## REDUCING ZINCIFEROUS MATERIALS CONTAINING LEAD

Application filed January 4, 1928. Serial No. 244,519.

This invention relates to the reduction or smelting of zinciferous materials containing lead and has for its object the provision of certain improvements in the smelting of such zinciferous materials whereby an effective elimination of lead is obtained.

Lead is one of the common contaminants of zinc ores and their concentrates, and when present in relatively small amounts prevents the production by pyrometallurgical methods of high grade zinc products, such as zinc metal, zinc oxide, zinc dust, etc., substantially free of lead. A relatively large tonnage of zinc concentrates containing from 0.05 to 15 5% of lead are available for zinc smelting, but no entirely satisfactory pyrometallurgical method has heretofore existed for producing substantially lead-free zinc products therefrom. The present invention is particularly applicable to the pyrometallurgical treatment of such zinc concentrates and other zinciferous materials containing lead, since by the practice of the invention high grade zinc products substantially free from 25 lead can be produced therefrom.

The gaseous product resulting from the smelting of a charge of zinciferous material containing lead consists for the most part of metallic zinc vapor, carbon monoxide, and a 30 small amount of lead. In the heretofore customary zinc smelting practices, any lead in the gaseous product will, for the most part, accompany the zinc vapor and thereby contaminates the final zinc product. Through 35 out this specification and the appended claims, we have used the word lead in a general sense and mean to embrace thereby not only metallic lead but compounds of lead. On the other hand, such lead-content figures 40 as are given in the specification are percentages of lead calculated as metallic lead.

In addition to lead, the zinc smelting charge may and usually does contain one or more other contaminating metals which, like 45 lead, boil at temperatures above the boiling temperature of zinc but which find their way into the gaseous product of the zinc smelting operation and thereby contaminate the zinc product obtained therefrom. While these 50 other contaminating metals, such, for exam-

ple as tin, antimony, bismuth, aluminum, magnesium, germanium and thallium, are ordinarily present in relatively small percentages, frequently amounting to mere traces, they very often deleteriously influence 55 the properties of the ultimate zinc product.

The object of our present invention is to provide a pyrometallurgical treatment for zinciferous materials containing one or more of the aforementioned contaminating metals 60 in the course of which a substantial removal of the contaminating metals is effected, thereby making possible the recovery of a purer and more desirable zinc product than can be obtained by the heretofore customary methods of zinc smelting. Since, in the practice 65 of the invention, all of the contaminating metals appear to behave similarly, we will herein more particularly describe the invention with respect to the elimination of lead. 70 The invention may be practiced solely for the elimination of lead without special regard to the elimination of other metals, or it may be practiced for the elimination of any one or more of the contaminating metals. In general, 75 the elimination of substantially all of the lead by the practice of the invention will at the same time effect a substantial elimination of such others of the contaminating metals as may be present in the zinc smelting charge. In the interests of conciseness the appended claims are directed particularly to lead removal, but we intend thereby to cover or include the removal of any one or more of the aforementioned contaminating metals. 80

The present invention is based on our discovery that lead can be almost completely removed from the gaseous product of the zinc smelting operation by passing the gaseous product through an eliminating or de-leading medium composed of at least one ingredient of the zinc smelting charge maintained under reducing conditions at an appropriate and carefully regulated elevated temperature. We have further found that 90 practical considerations make it desirable to supply the gaseous product to the de-leading medium in a substantially continuous stream of relatively constant volume and composition and practically free of oxidizing gases. 100

Based on these discoveries, the invention involves conducting the gaseous product resulting from the reduction or smelting of a charge of zinciferous material containing lead through a hot de-leading medium composed of at least one ingredient of the zinc reducing charge, preferably about to be subjected to the reducing operation, maintained at a regulated temperature sufficiently low to effect substantial elimination of lead from the gaseous product. The zinc reducing operation is preferably conducted so as to produce and supply to the de-leading medium a substantially continuous stream of the resulting gaseous product which should preferably be of relatively constant volume and composition and practically free of oxidizing gases. The de-leading medium is appropriately confined and arranged intermediate the zinc smelting chamber and the zinc recovery apparatus so that the de-leaded gaseous product passes, preferably in a substantially continuous stream, from the de-leading medium to the zinc recovery apparatus.

While the de-leading medium may be composed of any ingredient of the reducing charge, we prefer to employ the reducing charge itself consisting of the mixed zinciferous material and carbonaceous reducing agent. The de-leading medium should provide a multiplicity of tortuous paths for the flow therethrough of the gaseous product and should yet be sufficiently porous to permit the free passage of the gaseous product. These conditions are satisfactorily attained when the de-leading medium is composed of a body of aggregates. The aggregates may be naturally formed such as crushed or broken coke, coal or zinc ore, or may be artificially formed as by briquetting, sintering and the like. The aggregates should be approximately uniform in size in order that the porosity of the de-leading medium as a whole may be substantially uniform. Furthermore, in order to provide the desired multiplicity of tortuous gas passages, the aggregates should not be too large. We have secured very satisfactory results with a de-leading medium composed of briquettes approximately three inches in diameter or thickness confined in a vertically disposed cylinder about 15 inches internal diameter and about 6 feet long or high, where approximately one ton of zinc metal was recovered each 24 hours from the gaseous product passing through the de-leading medium.

It is our belief that the removal of lead by the eliminating medium is most effective, and probably only possible, when the lead is present in the reduced state. The de-leading medium must therefore be maintained under reducing conditions or in a reducing atmosphere free of any oxidizing influence, in order to inhibit the oxidation of metallic lead

and zinc, and, if necessary, to reduce any oxidized lead or zinc that might be present in the gaseous product. Should air or other oxidizing gas leak into or otherwise enter the enclosure for the de-leading medium, the effectiveness of the lead removal is seriously impaired, if not completely destroyed. Preferably, the reducing operation is conducted so that the gaseous product thereof consists mainly of carbon monoxide and metallic zinc vapor with only a fraction of a percent of carbon dioxide. Where the carbon dioxide content of the gaseous product of the reducing operation exceeds about 1 to 2%, the de-leading medium should contain the reducing agent of the reducing charge, such as coal, coke or the like, in order to insure the necessary reducing conditions in the de-leading medium for the effective removal of lead.

It is our preferred practice to maintain the de-leading medium at a carefully regulated temperature below the temperature at which lead compounds will be volatilized and at which any substantial amount of lead will remain with the gaseous product, under the prevailing conditions of operation. Such temperature regulation is essential where the de-leading medium is composed in whole or in part of zinciferous material in order to effect the desired lead elimination without substantial reduction of the zinciferous material of the de-leading medium. In practicing the invention we have secured very satisfactory results by maintaining the de-leading medium at a temperature intermediate the temperature at which zinc is reduced from its compounds and the temperature at which metallic zinc vapor is condensed, and of course below the temperature at which lead will remain with the gaseous product, under the prevailing operating conditions, whereby no substantial condensation of zinc vapor takes place in the de-leading medium.

The desired temperature regulation and control of the de-leading medium may be effected in any appropriate and convenient manner. This may be conveniently done by surrounding the de-leading medium with means for varying or adjusting the heat radiation therefrom. We have secured excellent results in practice by confining the de-leading medium in a vertical tube several feet in length and surrounded by heat insulating material of variable thickness or effectiveness. By appropriately adjusting the effectiveness of the heat insulating material, the radiation of heat from the tube can be so controlled as to maintain the desired temperature of the de-leading medium.

We have found that the character and composition of the gaseous product resulting from the zinc reducing operation has an important bearing on the effectiveness of the

removal of the lead in accordance with the principles of our invention. The best results are obtained when the gaseous product is a substantially continuous stream of zinc vapor and carbon monoxide relatively constant in volume and composition and practically free of oxidizing gases. Such a gaseous product may be advantageously obtained in the process of smelting an agglomerated or briquetted charge of zinciferous and reducing materials in accordance with the principles disclosed in the copending application of Messrs. Breyer and Bunce, Serial No. 163,902, filed January 27, 1927.

Where the process of the aforementioned Breyer and Bunce application is carried out in an upright or vertical retort, the improvements of the present invention may advantageously be embodied in the progress by providing an upper prolongation of the retort, above the reducing zone therein, adapted to confine the de-leading medium which in this case will be composed of a body or column of the agglomerated zinc smelting charge itself about to be advanced or introduced into the reducing zone of the retort. The agglomerated charge as a whole then progressively passes through the vertical retort and its prolongation and is heated in the reducing zone of the retort to a sufficiently high temperature to reduce compounds of zinc and volatilize the resulting metallic zinc and in the prolongation of the retort is maintained at an appropriate temperature to effect substantial removal of lead. The de-leading medium is thus superposed on the zinc-reducing charge undergoing reduction and, with appropriate renewal or introduction of fresh charge at the top, progressively descends from the de-leading zone to the smelting zone, and the worked-off or exhausted agglomerates are appropriately withdrawn from the bottom of the retort. The de-leaded gaseous product is withdrawn from the prolongation at or near the top of the de-leading body of agglomerates and is conducted to the zinc recovery apparatus, such as a condenser for zinc metal.

In the accompanying drawing, we have illustrated an apparatus adapted for the practice of the present invention in conjunction with the process of reducing zinciferous material disclosed in the aforementioned Breyer and Bunce application. It is to be understood that the drawing is illustrative, and that the invention may be practiced in other types or forms of apparatus. It is furthermore to be understood that the invention is not limited to this particular process of reducing zinciferous material, but is generally applicable to any smelting treatment of zinciferous material containing lead.

The single figure of the drawing is a sectional elevation of the upper portion of a vertically disposed smelting retort and aux-

iliaries for practicing the improvements of the invention. The vertical retort 5 is appropriately mounted within the heating chamber or laboratory 6 of an appropriate furnace structure 7. The retort may be heated by electric energy, by coal, oil or gas fuels or in any other appropriate manner. The retort 5 extends through the roof of the furnace structure 7 to a distance of several feet above the top of that structure thereby forming what may be termed an upper prolongation 5' of the retort. This upper prolongation may be integrally built with the retort proper or may be a separate unit superposed on top of the retort. The integral construction is preferred since joints and the possibility of air leakage into the retort are thereby avoided.

The prolongation 5' of the retort is surrounded by a layer 8 of heat insulating material, such as dust coal, appropriately confined by a surrounding sheet metal casing 9. Near the top of the prolongation 5' a gas off-take 10 is provided communicating with a condenser 11. The condenser illustrated in the drawing is of the multi-channel type comprising a gas distributing and molten metal collecting chamber 12 communicating with the lower ends of a multiplicity of upright channels 13. Condensers of this type are described in detail in the copending application of Frank G. Breyer, Serial No. 167,135, filed February 10, 1927.

The agglomerates of mixed zinciferous material and carbonaceous reducing agent are introduced into the vertical retort through an appropriate charging device (diagrammatically indicated by 14) at the top of the prolongation 5'. This charging device is of such construction that no air enters the top of the retort and little or none of the gaseous product escapes, and the agglomerates are introduced into the retort without blocking the gas off-take 10. The retort including its upper prolongation is filled with the agglomerated charge up to about the level of the gas off-take 10. The spent residues or worked-off charge are withdrawn from the bottom of the retort 5 in a continuous manner or at appropriate periodic intervals, thereby making room for the introduction, from time to time, of fresh agglomerates through the charging device 14.

The retort operates in substantially a continuous manner. That portion of the retort within the heating chamber 6 is subjected to a sufficiently high temperature to bring about the reduction of the compounds of zinc in the smelting zone of the retort and the volatilization of the resulting metallic zinc. The gaseous products of the reducing operation rise in the retort 5 and pass through the relatively cooler body of agglomerates confined in the prolongation 5'. These agglomerates are about to enter the smelting zone

of the retort 5 but while functioning as the de-leading medium are superposed on the main body of agglomerates undergoing reduction. The temperature of the body of agglomerates within the prolongation 5' is controlled, by increasing or diminishing the thickness of the insulating layer 8 or by other appropriate temperature regulating means, so as to maintain the agglomerates at a temperature sufficiently low to prevent volatilization of lead compounds and to effect substantial elimination of lead without condensing any substantial amount of zinc vapor. The thus de-leaded gases pass through the off-take 10 into the condenser 11 where substantially all of the zinc vapor is condensed to zinc metal.

The following specific example illustrates the principles of the present invention as practiced in an apparatus of the form shown in the accompanying drawing, although it is to be understood that this example is merely illustrative and in no sense restrictive of the invention.

The charges was made up of approximately 50 parts by weight of finely divided zinc ore (containing from 65-70% of zinc and 1.5 to 3.5% of lead) and 50 parts by weight of a bituminous coking coal. The zinc ore and coal were each crushed so that approximately 80% passed through a 20-mesh screen, and were then dumped into a dry pan Chilian mill and subjected to the mixing and comminuting action of the mill for some minutes. From the Chilian mill, the mixed material was taken to a brietting press and formed into semi-round briquettes by a compressive force of approximately 2000 pounds to the square inch.

The briquettes, without drying, were charged into an externally heated vertical coking retort. In this retort the briquettes were subjected to a coking temperature of about 950° C. for about 1½ hours. The coked briquettes were transferred without substantial loss of heat from the coking retort to the prolongation 5' of the vertical smelting retort and introduced therein at the rate of approximately 180 pounds at intervals of 45 minutes. The temperature within the heating chamber 6 was about 1100 to 1250° C., and the body of de-leading agglomerates in the prolongation 5' was maintained at a temperature of about 800 to 900° C. In the particular example being discussed, the retort 5 was about 25 feet long (high) and slightly over 15 inches internal diameter, while the prolongation 5' was about 8 feet long. The retort 5 and prolongation 5' were built as a unitary structure of silicon carbide circle brick, supported solely at the base and not otherwise tied into the furnace structure.

The upper level of the briquetted charge was maintained at the level of the condenser off-take 10. This was accomplished by with-

drawing from the bottom of the retort 5 an appropriate amount of worked-off briquettes while charging fresh briquettes into the top of the retort. The column or body or briquettes in the prolongation 5' of the retort above the top of the furnace structure 7 was approximately 6 feet in height.

The gaseous product of the reducing operation taking place in the highly heated portion of the retort 5 was conducted through the superposed body or column of relatively cooler briquettes in the prolongation 5' and thence through the off-take 10 to the condenser 11. This gaseous product consists for the most part of metallic zinc vapor, carbon monoxide gas and small percentages of lead, and of itself provides a strongly reducing atmosphere within the prolongation 5'. In passing through the column of de-leading briquettes in the prolongation 5' substantially all of the lead was removed from the gaseous product and remained with the de-leading briquettes. In the example under discussion, the lead content of the zinc metal collected in the condenser 11 varied from 0.019 to 0.050%. Operating under the same conditions, except that the upper level of the briquetted charge in the retort is maintained at about the level of the arch of the furnace structure 7, the lead content of the condensed zinc metal varies from 0.5 to 1.25%. Likewise, working this same ore in an ordinary zinc distillation furnace in accordance with the customary spelter retort practice, the resulting zinc metal contains 1% lead and over.

Applying the principles of the invention to a zinc ore containing a relatively small amount of lead, smelted in accordance with the method of the invention just described, we have succeeded in producing zinc metal containing from 0.0024 to 0.0032% lead. Treating this same ore by the same procedure, but maintaining the charge level in the retort at about the level of the furnace arch, the resulting zinc metal contains from 0.08 to 0.12% lead. Likewise, in treating this same ore in accordance with the present spelter retort practice, the resulting zinc metal contains from 0.08 to 0.12% lead.

The lead removed from the gaseous product of the smelting operation by the de-leading body of agglomerates accompanies the agglomerates into the smelting zone of the retort in a condition or form less readily returned to the gaseous product than the condition or form in which the lead occurs in the zinciferous material. Just what happens to this lead in the smelting zone, we are not prepared to say, but it, in large part at least, passes out of the bottom of the retort with the worked-off residues. Whatever the correct explanation of the phenomenon may be, the facts themselves are clear, and almost complete de-leading of the gaseous product is effected in its passage through the tempera-

ture-controlled de-leading body of agglomerates.

It will be clear from the foregoing description that careful regulation and control of the temperature of the body of de-leading agglomerates, or other form of zinciferous and/or carbonaceous material of the smelting charge, is essential for the effective elimination of lead without the condensation of any substantial amount of zinc vapor. This temperature regulation and control is most advantageously accomplished in the apparatus illustrated in the drawing by controlling the heat radiation from the prolongation 5'. This may be conveniently done by providing the sheet metal casing 9 with doors, or the like, through which the dust coal insulation 8 surrounding the prolongation 5' may be increased or diminished. Other appropriate means of temperature regulation and control may be used. The temperature of the gases within the prolongation 5' is determined by appropriately positioned pyrometers or other heat measuring instruments.

The advantages of the invention will be manifest to those skilled in the art. The lead elimination is effected by the smelting charge itself, and preferably just preceding its introduction into the reducing chamber. By superposing the de-leading body of charge on the charge undergoing reduction, all extraneous apparatus is avoided and joints or mechanical connections through which air might leak into the system are eliminated. Furthermore, the superposed column of de-leading agglomerates provides a relatively long path for the de-leading operation, and affords excellent opportunity for close temperature control.

It is important that the de-leading body of charge be maintained in a reducing atmosphere free of any oxidizing influences. To prevent air or oxidizing gases being carried into the prolongation 5' during the introduction of fresh charge, it is our preferred practice to introduce the charge into the prolongation 5' at a temperature at which there is sufficient gas evolution from the fresh charge to prevent the entraining of air. Should air or other oxidizing gas leak into or otherwise enter the de-leading body of charge, the effectiveness of the lead removal will be seriously impaired, if not completely destroyed. This is one of the chief advantages resulting from our preferred unitary construction of the retort 5 and prolongation 5', since air leakages are thereby effectively inhibited.

While in our preferred practice, the de-leading medium is composed of the mixed reducing or smelting charge, the medium may, if desired, be composed of any ingredient of the reducing charge, such as the zinciferous material alone, or the reducing agent alone. Again, while it is our preferred prac-

tice to superpose the de-leading medium on the charge undergoing smelting, thereby simplifying the operation and facilitating renewal of the de-leading medium, other ways of confining the de-leading medium and of renewing the medium from time to time may be employed. We consider it advantageous to progressively move the de-leading medium in a direction opposite to that of the direction of flow of the gaseous product, and to renew the medium from time to time by fresh de-leading material added thereto at a temperature approximating the temperature at which the medium is maintained. Furthermore, while it is our preferred practice to conduct the de-leading without substantial condensation of metallic zinc vapor in the de-leading medium, this is not essential, since whatever zinc is condensed in the de-leading medium is readily revolatilized and recovered, particularly when the de-leading medium is next subjected to the smelting operation where the condensed zinc is revolatilized and returned to the gaseous product.

While we have particularly described the recovery of the metallic zinc vapor from the de-leaded gaseous product in the form of zinc metal or spelter, it is to be understood that the vapor may be recovered in other forms of zinc products. Thus, the zinc vapor may be condensed as zinc dust, or may be oxidized and collected as zinc oxide. In any case, the practice of the invention enables the production of zinc products more nearly lead-free than could otherwise be obtained by pyrometallurgical methods from the lead-containing zinc ores.

We claim:

1. The improvement in the reduction of zinciferous material containing lead which comprises conducting the gaseous product of the reducing operation through a hot body of the reducing charge maintained at a regulated temperature sufficiently low to effect substantial removal of lead from said gaseous product, and subjecting the thus de-leaded gaseous product to appropriate treatment for the recovery of the zinc content thereof.

2. The improvement in the reduction of zinciferous material containing lead which comprises conducting the gaseous product of the reducing operation through a body of the reducing charge maintained at a temperature of from 800 to 900° C. and thereby effecting substantial removal of lead from said gaseous product, and subjecting the thus de-leaded gaseous product to appropriate treatment for the recovery of the zinc content thereof.

3. The improvement in the reduction of zinciferous material containing lead which comprises conducting the gaseous product of the reducing operation through a hot body of the reducing charge about to be subjected to the reducing operation and maintained at a

regulated temperature sufficiently low to effect substantial removal of lead from said gaseous product, and subjecting the thus de-leaded gaseous product to appropriate treatment for the recovery of the zinc content thereof.

4. The improvement in the reduction of zinciferous material containing lead which comprises conducting the gaseous product of the reducing operation through a hot body of the reducing charge about to be subjected to the reducing operation and maintained at a regulated temperature sufficiently low to effect substantial removal of lead from said gaseous product, progressively moving said de-leading body of the reducing charge in a direction opposite to the direction of flow of the gaseous product therethrough, and subjecting the thus de-leaded gaseous product to appropriate treatment for the recovery of the zinc content thereof.

5. The improvement in the reduction of zinciferous material containing lead which comprises conducting the gaseous product of the reducing operation through a hot body of the reducing charge about to be subjected to the reducing operation and maintained at a regulated temperature sufficiently low to effect substantial removal of lead from said gaseous product, renewing said de-leading body of the reducing charge from time to time by fresh reducing charge added thereto at a temperature approximating that at which the de-leading body of charge is maintained, and subjecting the thus de-leaded gaseous product to appropriate treatment for the recovery of the zinc content thereof.

6. The improvement in the reduction of zinciferous material containing lead which comprises conducting the gaseous product of the reducing operation through a hot body of the reducing charge about to be subjected to the reducing operation and maintained at a regulated temperature sufficiently low to effect substantial removal of lead from said gaseous product, progressively moving said de-leading body of the reducing charge in a direction opposite to the direction of flow of the gaseous product therethrough, renewing said de-leading body of the reducing charge from time to time by fresh reducing charge added thereto at a temperature approximating that at which the de-leading body of charge is maintained, and subjecting the thus de-leaded gaseous product to appropriate treatment for the recovery of the zinc content thereof.

7. The improvement in the reduction in an externally heated upright retort of an agglomerated charge of carbonaceous reducing agent and zinciferous material containing lead which comprises conducting the gaseous product of the reducing operation through a body of fresh agglomerates about to be subjected to the reducing operation and main-

tained at a temperature sufficiently low to effect substantial removal of lead from said gaseous product without condensing any substantial amount of zinc vapor, and subjecting the thus de-leaded gaseous product to appropriate treatment for the recovery of the zinc content thereof.

8. The improvement in the reduction of zinciferous material containing lead which comprises subjecting coked agglomerates of the zinciferous material and a carbonaceous reducing agent to a reducing operation, conducting the gaseous product of the reducing operation through a hot body of the coked agglomerates maintained at a regulated temperature sufficiently low to effect substantial removal of lead from said gaseous product, and subjecting the thus de-leaded gaseous product to appropriate treatment for the recovery of the zinc content thereof.

9. The improvement in the reduction of zinciferous material containing lead which comprises progressively passing a charge of the zinciferous material and an appropriate reducing agent through a reducing chamber heated to a sufficiently high temperature to reduce compounds of zinc and volatilize the resulting metallic zinc, conducting the gaseous product of the reducing operation through a body of fresh charge about to be introduced into said reducing chamber and maintained at a regulated temperature sufficiently low to effect substantial removal of lead from said gaseous product, and subjecting the thus de-leaded gaseous product to appropriate treatment for the recovery of the zinc content thereof.

10. The improvement in the reduction of zinciferous material containing lead which comprises progressively passing an agglomerated charge of the zinciferous material and carbonaceous reducing agent through a reducing chamber heated to a sufficiently high temperature to reduce compounds of zinc and volatilize the resulting metallic zinc, conducting the gaseous product of the reducing operation through a body of fresh agglomerates about to be introduced into said reducing chamber and maintained at a temperature sufficiently low to effect substantial removal of lead from said gaseous product without condensing any substantial amount of zinc vapor, and subjecting the thus de-leaded gaseous product to appropriate treatment for the recovery of the zinc content thereof.

11. The improvement in the reduction of zinciferous material containing lead which comprises progressively passing a charge of the zinciferous material and an appropriate reducing agent through an upright reducing chamber in which the charge is heated to a sufficiently high temperature to reduce compounds of zinc and volatilize the resulting metallic zinc, conducting the gaseous product of the reducing operation through a hot body

5 of fresh charge confined in a prolongation of the reducing chamber and superposed on the charge undergoing reduction and maintained at a regulated temperature sufficiently low to effect substantial removal of lead from said gaseous product, and subjecting the thus de-leaded gaseous product to appropriate treatment for the recovery of the zinc content thereof.

10 12. The improvement in the reduction of zinciferous material containing lead which comprises progressively passing a charge of the zinciferous material and an appropriate reducing agent through an upright retort in one portion of which the charge is heated to a sufficiently high temperature to reduce compounds of zinc and volatilize the resulting metallic zinc, and in another portion of which the gaseous product of the reducing operation is 15 conducted through a hot body of fresh charge superposed on the charge undergoing reduction and maintained at a regulated temperature sufficiently low to effect substantial removal of lead from said gaseous product, introducing fresh charge into the top of said retort at a temperature approximating the temperature maintained in said superposed de-leading body of charge, and subjecting the thus de-leaded gaseous product to appropriate 20 treatment for the recovery of the zinc content thereof.

25 13. The improvement in the reduction of zinciferous material containing lead which comprises progressively passing an agglomerated charge of the zinciferous material and an appropriate reducing agent through an upright reducing chamber in which the charge is heated to a sufficiently high temperature to reduce compounds of zinc and volatilize the 30 resulting metallic zinc, conducting the gaseous product of the reducing operation through a hot body of fresh agglomerates confined in a prolongation of the reducing chamber and superposed on the charge undergoing reduction and maintained at a temperature sufficiently low to effect substantial removal of lead from said gaseous product, and subjecting the thus de-leaded gaseous product to appropriate treatment for the recovery of the 35 zinc content thereof.

40 14. The improvement in the reduction of zinciferous material containing lead which comprises progressively passing an agglomerated charge of the zinciferous material and a carbonaceous reducing agent through a vertical retort in one portion of which the charge is heated to a sufficiently high temperature to reduce compounds of zinc and volatilize the resulting metallic zinc and in another portion 45 of which the gaseous product of the reducing operation is conducted through a body of fresh charge superposed on the charge undergoing reduction and maintained at a regulated temperature sufficiently low to effect 50 substantial removal of lead from said gaseous product without condensing any substantial amount of zinc vapor, and subjecting the thus de-leaded gaseous product to appropriate treatment for the recovery of the zinc content thereof.

55 15. The improvement in the reduction of zinciferous material containing lead which comprises progressively passing an agglomerated charge of the zinciferous material and an appropriate reducing agent through an upright reducing chamber in which the charge is heated to a sufficiently high temperature to reduce compounds of zinc and volatilize the resulting metallic zinc, conducting the gaseous product of the reducing operation through a hot body of fresh agglomerates confined in a prolongation of the reducing chamber and superposed on the charge undergoing reduction and maintained at a temperature sufficiently low to effect substantial removal of lead from said gaseous product, introducing fresh agglomerates into said prolongation at a temperature approximating the temperature maintained in said superposed de-leading body of agglomerates, and subjecting the thus de-leaded gaseous product to appropriate treatment for the recovery of the zinc content thereof.

60 In testimony whereof we affix our signatures.

EARL H. BUNCE.  
GEORGE T. MAHLER.

70

75

80

85

90

95

100

105

110

115

120

125

130